

## UNITED STATES PATENT OFFICE

2,262,690

## PRODUCTION OF FREE-MACHINING STAIN-LESS STEEL

Vincent T. Malcolm, Indian Orchard, Mass., assignor to The Chapman Valve Manufacturing Co., Indian Orchard, Mass., a corporation of Massachusetts

No Drawing. Application June 22, 1940,  
Serial No. 341,961

2 Claims. (Cl. 148—21.5)

This invention relates to improvements in producing a free-machining so-called 11-14% chromium steel having a relatively low sulphur content and is directed more particularly to the provision of a free-machining 11-14 chromium steel having all the desirable characteristics inherent in steels of the same type which have a relatively high sulphur content but none of their disadvantages.

It has for some time been the practice to make chromium steels for use in the manufacture of such machined parts as valve stems, other valve parts, etc., by means of such machines as so-called automatic screw machines which operate at high speeds, but success has only been had, as far as efficiency, speed, and economy are concerned, when these steels have had a relatively high sulphur content, say around .25 to .50%. However, the oil, chemical, and other industries which employ machined steel parts under such conditions that they are subjected to the action of various gases and acids at high temperatures have for some time objected to the corrosiveness and high degree of brittleness in such steels.

That is to say, while 11-14 chromium steels having this relatively high sulphur content are capable of rapid and efficient machining, the sulphur content at the same time has been more or less of a contaminating element wherefore such steels are not satisfactory for use in these industries.

Other chromium steels containing relatively less sulphur have, of course, been produced but they are not readily adapted for machining in automatics. That is to say, 11-14 chromium steels containing a relatively low amount of sulphur have been made but they have never been used with success in automatic machines which operate at high speeds since the cutting speed of such low-sulphur chromium steels is about 30 feet per minute as contrasted with a cutting speed of around 100 feet per minute of a chromium steel containing a larger amount of sulphur.

Further, the outside threading and finishing of a chromium steel having a low sulphur content on an automatic high-speed machine is rough and of poor quality and tapping thereon is practically impossible. That is, such steels have had to be removed from the automatic machines and tapped and threaded by more or less of a hand method.

It is, accordingly, the principal object of this invention to provide a 11-14% chromium steel which does not have the corrosive or objectionably brittle qualities of such steels containing the

relatively high amount of sulphur but which has their fine machining qualities. In other words, by the method of this invention, I take a 11-14% chromium steel having a low sulphur content and give to it the machining properties of a similar steel having a higher sulphur content while eliminating the contaminating influence thereof.

The formula of a common 11-14% chromium steel having a relatively high sulphur content and which has met with success as far as its machinability is concerned, is as follows:

|                        |                  |            |
|------------------------|------------------|------------|
| Carbon                 | per cent maximum | .15        |
| Manganese              | do               | .50        |
| Silicon                | do               | .50        |
| Phosphorus             | do               | .04        |
| Nickel                 | do               | .50        |
| Chromium               | do               | 11.5-13.0  |
| Sulphur, approximately | per cent         | .25 to .50 |

As stated, however, such steels are not adapted for use in oil refineries, for example, where the machined valve stems or the like must withstand the action of acids and gases at elevated temperatures. According to this invention, I employ a steel having the same approximate formula set forth above except that the sulphur content of the steel I work preferably has a maximum sulphur content of .05%.

The preferred process of heat treating this type of steel will now be described.

The piece or pieces are first heated slowly in a suitable furnace to a temperature below the critical transformation point of the steel preferably to about 1450° F. The steel is soaked or held at this temperature until the heat penetration is substantially complete, this usually taking about one and one-half hours for each inch of thickness.

After this the pieces are heated rapidly to a higher temperature which, nevertheless, is still below a temperature at which the carbides have not gone completely into solution and preferably between 1550° F. and 1625° F., from which temperature the steel is then cooled rapidly, either in air or oil.

It will be noted that all heating is at a temperature below the complete carbide solution point. The steel is brought to a uniform heat condition throughout at a temperature of approximately 1450° F. without the danger of excessive grain size formation and then it is quickly brought to about 1580° F. where it is rapidly cooled or quenched in air or oil.

The above process has the advantages of providing really machinable 11-14 chromium steels,

as contrasted with stainless steels hitherto made which are too hard or tough for my purposes. Further, according to this invention more uniform results can be obtained, especially inasmuch as a whole batch of pieces may be quenched simultaneously with uniformity.

It will also be obvious that any subsequent heat-treating steps are not always necessary and that my process, being relatively simple and easy to perform, requires less care in its operation. Thus it is more economical.

Manifestly the specific details of construction may be considerably varied from those herein shown and described without involving any departure from the principle of the invention or sacrificing any of the advantages inherent therein. While I have described my invention in this specification in great detail and particularly with respect to the present preferred form thereof, it is not desired to be limited thereto since many changes and modifications may be made therein without departing from the spirit and scope of the invention.

The invention may be embodied in other specific forms without departing from the essential characteristics thereof. Hence, the present embodiments are therefore to be considered in all respects merely as being illustrative and not as being restrictive, the scope of the invention being indicated by the appended claims

rather than by the foregoing description, and all modifications and variations as fall within the meaning and purview and range of equivalency of the appended claims are therefore intended to be embraced therein.

What it is desired to claim and secure by Letters Patent of the United States is:

1. The process of treating 11-14% chromium steel so as to render the same free-machining which consists in, heating the steel to a temperature below its critical temperature point and around 1450° F., then stepping up the heat to a temperature around 1580° F., and finally quenching the steel rapidly, whereby the structure produced is partially martensitic together with carbides and the steel is in a semi-hardened condition.

2. The process of treating 11-14% chromium steel so as to render the same free-machining which consists in, heating the steel to a temperature below its critical transformation point and around 1450° F., then stepping up the heat to a temperature which is still below the complete carbide solution point and around 1580° F., and finally quenching the steel rapidly, whereby the structure produced will be partially martensitic together with carbides and the steel is in a semi-hardened condition.

VINCENT T. MALCOLM.